

# United States Patent

[19]

Salsgiver et al.

[11] 3,855,021

[45] Dec. 17, 1974

[54] PROCESSING FOR HIGH PERMEABILITY  
SILICON STEEL COMPRISING COPPER

[75] Inventors: James A. Salsgiver, Sarver; Frank A. Malagari, Freeport, both of Pa.

[73] Assignee: Allegheny Ludlum Industries, Inc., Pittsburgh, Pa.

[22] Filed: May 7, 1973

[21] Appl. No.: 358,238

[52] U.S. Cl. .... 148/112, 75/123 L, 148/31.55,

148/111

[51] Int. Cl. .... H01f 1/04

[58] Field of Search .... 148/112, 111, 110, 31.55;  
75/123 L

## [56] References Cited

### UNITED STATES PATENTS

|           |         |                 |         |
|-----------|---------|-----------------|---------|
| 3,159,511 | 12/1964 | Taguchi et al.  | 148/111 |
| 3,287,184 | 11/1966 | Koh             | 148/113 |
| 3,345,219 | 10/1967 | Detert          | 148/112 |
| 3,632,456 | 1/1972  | Sakakura et al. | 148/111 |
| 3,671,337 | 6/1972  | Kumai et al.    | 148/112 |

## OTHER PUBLICATIONS

Lyman, T., Metals Handbook, ASM, Cleveland, 1948, p. 628, (TA472 A3).

Kussmann, A., et al., Gekupferter Stahl For ... Transform., in Stahl and Eisen, 50, (1930), pp. 1194-1197, (TS300 S7).

Primary Examiner—Walter R. Satterfield

Attorney, Agent, or Firm—Vincent G. Giola; Robert F. Dropkin

## [57] ABSTRACT

A process for producing silicon steel having a cube-on-edge orientation and a permeability of at least 1850 (G/O<sub>e</sub>) at 10 oersteds, which includes the steps of: cold rolling silicon steel; annealing the cold rolled steel prior to a final cold roll, at a temperature of from 1400° to 1700°F for a period of from 15 seconds to 2 hours; cooling the annealed steel at a rate substantially equivalent to a still air cool; and cold rolling the cooled steel at a reduction of at least 80 percent.

12 Claims, No Drawings

**PROCESSING FOR HIGH PERMEABILITY  
SILICON STEEL COMPRISING COPPER**

The present invention relates to a process for producing electromagnetic silicon steel having a cube-on-edge orientation and a permeability of at least 1850 (G/O<sub>e</sub>) at 10 oersteds.

Oriented silicon steels containing 2.60 to 4.0 percent silicon are generally produced by processes which involve hot rolling, a double cold reduction, an anneal before each cold roll and a high temperature texture anneal. Characterizing these steels are permeabilities at 10 oersteds of from 1790 to 1840 (G/O<sub>e</sub>).

In recent years a number of patents have disclosed silicon steels with permeabilities in excess of 1850 (G/O<sub>e</sub>) at 10 oersteds. Of these, U.S. Pat. Nos. 3,287,183, 3,632,456 and 3,636,579 appear to be the most interesting from a processing standpoint. U.S. Pat. No. 3,287,183 which issued on Nov. 22, 1966 reveals that a steel composed of specific amounts of carbon, silicon, aluminum, sulfur and iron could be processed into a high permeability silicon steel by cold rolling from 5 to 40 percent, annealing at a temperature of from 1742° to 2192°F so as to precipitate AlN, cold rolling from 81 to 95 percent, decarburizing and final texture annealing. More recently, similar processing for similar alloys was disclosed in U.S. Pat. Nos. 3,632,456 and 3,636,579, which respectively issued on Jan. 4, 1972 and Jan. 25, 1972. Each of these patents refer to cooling rates following the anneal in which AlN is precipitated. U.S. Pat. No. 3,632,456 anneals a hot rolled band at a temperature of from 1382° to 2192°F depending upon its silicon content, rapidly cools the annealed band and then proceeds to subject it to at least two cold rollings. U.S. Pat. No. 3,636,579 anneals steel containing 2.5 to 4.0 percent silicon at a temperature of from 1742° to 2192°F, quenches it from said temperature to a temperature at least as low as 752° F and then cold rolls it.

Described herein is another, and improved method for producing silicon steel having a cube-on-edge orientation and a permeability of at least 1850 (G/O<sub>e</sub>) at 10 oersteds from steel of a particular chemistry. The method includes the steps of: cold rolling silicon steel; annealing the cold rolled steel prior to a final cold roll, at a temperature of from 1400° to 1700°F for a period of from 15 seconds to 2 hours; cooling the annealed steel at a rate substantially equivalent to a still air cool; and cold rolling the cooled steel at a reduction of at least 80 percent. It differs and is contradictory to the methods of heretofore referred to U.S. Pat. Nos. 3,287,183, 3,632,456 and 3,636,579 in that: U.S. Pat. No. 3,287,183 discloses a minimum annealing temperature of 1742°F and not a maximum annealing temperature of 1700°F; U.S. Pat. No. 3,632,456 calls for a hot rolled band anneal at a temperature in excess of 1742°F for steels containing at least 2.5 % Si and a rapid cool therefrom; and U.S. Pat. No. 3,636,579 discloses a minimum annealing temperature of 1742°F for steels containing at least 2.5% Si and a rapid cool from said annealing temperature. Moreover, the chemistry of the steel being processed in accordance with the present invention differs from that being processed in said heretofore referred to patents.

It is accordingly an object of the present invention to provide a process for producing electromagnetic silicon steel having a cube-on-edge orientation and a permeability of at least 1850 (G/O<sub>e</sub>) at 10 oersteds.

The present invention provides a method for producing silicon steel having a cube-on-edge orientation and a permeability of at least 1850 (G/O<sub>e</sub>), and preferably at least 1900 (G/O<sub>e</sub>), at 10 oersteds. Involved therein are the steps of: preparing a melt of silicon steel having, by weight, up to 0.07% carbon, from 2.60 to 4.0% silicon, from 0.03 to 0.24% manganese, from 0.01 to 0.07% sulfur, from 0.015 to 0.04% aluminum, up to 0.02% nitrogen, and from 0.1 to 0.5% copper; casting the steel; hot rolling the steel into a hot rolled band, cold rolling the hot rolled band with or without an intermediate anneal between the hot rolling and the cold rolling, the intermediate anneal being at a maximum temperature of 1700°F; subjecting the steel to at least one additional cold rolling; subjecting the steel to a final annealing prior to the final cold rolling; decarburizing the steel; and final texture annealing the steel. Also included, and significantly so, are the specific steps of: carrying out the final anneal prior to the final cold rolling at a temperature of from 1400° to 1700°F for a period of from 15 seconds to 2 hours; cooling the annealed steel at a rate substantially equivalent to a still air cool; and cold rolling the cooled steel at a reduction of at least 80 percent. Preferred conditions include annealing at a temperature of from 1450° to 1650°F and cold rolling at a reduction of at least 85 percent. For purposes of definition, still air cools include those wherein the steel is cooled in a static atmosphere as well as those wherein there is relative motion between the atmosphere and the steel, as in a continuous processing line, so long as there is no deliberate intention to cause the motion for cooling purposes. Moreover, for purposes of definition, all gaseous atmospheres are considered to have the same cooling effect as air. Hence, all open cools are at a rate substantially equivalent to a still air cool unless a liquid quenching medium or forced gaseous atmosphere is employed, and a forced gaseous atmosphere is one in which motion is deliberately imparted to the atmosphere for cooling purposes.

Melting, casting, hot rolling, annealing, cold rolling, decarburizing and final texture annealing do not involve any novel procedures, as far as techniques are concerned, and with regard to them, the invention encompasses all applicable steel making procedures. Annealing at a temperature of from 1400° to 1700°F for the final anneal prior to the final cold roll is, however, believed to be particularly beneficial in that it conditions the steel for cold rolling, provides an operation during which inhibitors can form, and most importantly, increases the uniformity in which the inhibitors are distributed as essentially only ferrite phase is present in the steel at temperatures below 1700°F, contrasted to the presence of austenite and ferrite phases and different solubilities for the inhibiting elements in each phase at somewhat higher temperatures. By inhibitors, the invention primarily pertains to aluminum nitride, and manganese sulfide and/or manganese copper sulfide, which are discussed in greater detail hereinbelow. No criticality is placed upon the particular annealing atmosphere. Illustrative atmospheres therefore include nitrogen; reducing gases such as hydrogen; inert gases such as argon; air; and mixtures thereof. For similar reasons, as with the final anneal prior to the final cold roll the hot rolled band should not be annealed at temperatures in excess of 1700°F; and when a hot rolled band anneal is desired it is preferred to carry it

out at a temperature of from 1400° to 1700°F. The annealed hot rolled band is generally cooled at a rate substantially equivalent to a still air cool. As to the cold rolling, it should be pointed out that several roll passes can constitute a single cold rolling operation, and that plural cold rolling operations exist only when cold rolling passes are separated by an anneal.

The steel melt must include a silicon, aluminum, manganese, sulfur and copper. Silicon is necessary as it increases the steel's resistivity, decreases its magnetostriction, decreases its magnetocrystalline anisotropy and hence decreases its core loss. Aluminum, manganese and sulfur are necessary as they form inhibitors which are essential to controlling the steel's orientation and its properties which are dependent thereon. More specifically, aluminum combines with nitrogen, in the steel or from the atmosphere, to form aluminum nitride, and manganese combines with sulfur to form manganese sulfide and/or manganese copper sulfide; and these compounds act so as to inhibit normal grain growth during the final texture anneal, while at the same time, aiding in the development of secondary recrystallized grains having the desired cube-on-edge orientation. Copper in addition to possibly forming manganese copper sulfide, is believed to be beneficial in that it is hypothesized that copper can lower the annealing temperature, improve rollability, simplify melting and relax annealing atmosphere requirements.

A steel in which the process of the present invention is particularly adaptable to consists essentially of, by weight, from 0.02 to 0.07% carbon, from 2.60 to 3.5% silicon, a manganese equivalent of from 0.05 to 0.24% as expressed by an equivalency equation of %Mn + (0.1 to 0.25) × %Cu, from 0.01 to 0.05% sulfur, from 0.015 to 0.04% aluminum, from 0.0030 to 0.0090% nitrogen, from 0.1 to 0.3% copper, balance iron and residuals; and wherein the ratio of manganese equivalent to sulfur is in the range of from 2.0 to 4.75. The steel has its chemistry balanced so as to produce a highly beneficial structure when processed according to the present invention.

The following examples are illustrative of several aspects of the invention.

Five samples (Samples 1 - 5) of silicon steel were cast and processed into silicon steel having a cube-on-edge orientation from 5 different heats of BOF silicon steel. The chemistry of the samples appears hereinbelow in Table I.

ture of nitrogen and wet hydrogen, and final annealing for 8 hours in hydrogen at a maximum temperature of 2150°F.

Samples 1 - 5 were tested for permeability and core loss. The results of the tests appear hereinbelow in Table II.

TABLE II

|    | Sample | Permeability<br>-alkoxypropionyl<br>10 Oe) | Core Loss<br>(WPP at 17 KB) |
|----|--------|--------------------------------------------|-----------------------------|
| 10 | 1      | 1878                                       | 0.798                       |
|    | 2      | 1903                                       | 0.763                       |
|    | 3      | 1879                                       | 0.823                       |
|    | 4      | 1886                                       | 0.766                       |
|    | 5      | 1889                                       | 0.757                       |

From Table II, it is clear that the processing of the present invention is highly beneficial to the properties of silicon steel having a cube-on-edge orientation. Samples 1 through 5 were cold rolled, annealed at a temperature of 1475°F for 5 minutes, air cooled to room temperature and cold rolled in excess of 80%; and all had permeabilities in excess of 1850 (G/O<sub>e</sub>) at 10 O<sub>e</sub>. Moreover, sample 2 had a permeability in excess of 1900 (G/O<sub>e</sub>).

It will be apparent to those skilled in the art that the novel principles of the invention disclosed herein in connection with specific examples thereof will suggest various other modifications and applications of the same. It is accordingly desired that in construing the breadth of the appended claims they shall not be limited to the specific examples of the invention described herein.

We claim:

1. In a process for producing electromagnetic silicon steel having a cube-on-edge orientation and a permeability of at least 1850 G/O<sub>e</sub>) at 10 oersteds, which process includes the steps of: preparing a melt of silicon steel consisting essentially of, by weight, up to 0.07% carbon, from 2.60 to 4.0% silicon, from 0.03 to 0.24% manganese, from 0.01 to 0.07% sulfur, from 0.015 to 0.04% aluminum, up to 0.02% nitrogen, from 0.1 to 0.5% copper and the balance iron; casting said steel; hot rolling said steel into a hot rolled band; cold rolling said hot rolled band with or without an intermediate anneal between said hot rolling and said cold rolling, said intermediate anneal being at a maximum temperature of 1700°F; subjecting said band to at least one ad-

TABLE I

| Sample | C     | Mn    | COMPOSITION (Wt. %) |      |       |      |        |      |
|--------|-------|-------|---------------------|------|-------|------|--------|------|
|        |       |       | S                   | Si   | Al    | Cu   | N      | Fe   |
| 1      | 0.050 | 0.13  | 0.044               | 3.04 | 0.023 | 0.23 | 0.0039 | Bal. |
| 2      | 0.055 | 0.13  | 0.043               | 2.92 | 0.029 | 0.19 | 0.0055 | Bal. |
| 3      | 0.050 | 0.11  | 0.030               | 2.92 | 0.023 | 0.19 | 0.0055 | Bal. |
| 4      | 0.048 | 0.076 | 0.026               | 2.84 | 0.029 | 0.23 | 0.0041 | Bal. |
| 5      | 0.049 | 0.094 | 0.032               | 2.91 | 0.036 | 0.22 | 0.0046 | Bal. |

Processing for the five samples involved soaking at an elevated temperature for several hours, blooming, hot rolling to a gage of approximately 130 mils, normalizing for 2 minutes at 1650°F in air, cold rolling to a gage of approximately 92 mils, annealing at 1475°F for 5 minutes in impure nitrogen (nitrogen with approximately 0.1 to 10% oxygen), air cooling to room temperature; cold rolling to final gage of approximately 13 mils, decarburizing for 2 minutes at 1475°F in a mix-

60 ditional cold rolling; subjecting said band to a final annealing prior to the final cold rolling; decarburizing said steel; and final texture annealing said steel; the improvement comprising the steps of carrying out said final anneal prior to the final cold rolling at a temperature of from 1400° to 1700°F for a period of from 15 seconds to 2 hours; cooling said annealed steel at a rate equivalent to a still air cool, said cool including those wherein the steel is cooled in a static atmosphere or in

a continuous processing line where there is some relative motion between the atmosphere and the steel, and excluding furnace cools and those where relative motion is deliberately induced for cooling purposes; and cold rolling said cooled steel at a reduction of at least 80 percent.

2. An improvement according to claim 1, wherein said final anneal prior to the final cold rolling is at a temperature of from 1450° to 1650°F.

3. An improvement according to claim 1, wherein said cooled steel is cold rolled at a reduction of at least 85 percent.

4. An improvement according to claim 1, wherein the hot rolled band is cold rolled without an intermediate anneal between hot rolling and cold rolling.

5. An improvement according to claim 1, wherein the hot rolled band is annealed at a temperature of from 1400°-1700°F prior to being cold rolled.

6. An improvement according to claim 5, wherein said annealed hot rolled band is cooled at a rate equivalent to a still air cool prior to being cold rolled.

7. An improvement according to claim 1, wherein said steel consists essentially of, by weight, from 0.02 to 0.07% carbon, from 2.60 to 3.5% silicon, a manga-

5

nese equivalent of from 0.05 to 0.24%, as expressed by an equivalency equation of  $\%Mn + (0.1 \text{ to } 0.25) \times \%Cu$ , from 0.01 to 0.05% sulfur, from 0.015 to 0.04% aluminum, from 0.0030 to 0.0090% nitrogen, from 0.1 to 0.3% copper, balance iron and residuals; and wherein the ratio of manganese equivalent to sulfur is in the range of from 2.0 to 4.75.

8. An improvement according to claim 7, wherein said final anneal prior to the final cold rolling is at a temperature of from 1450° to 1650°F.

9. An improvement according to claim 7, wherein said cooled steel is cold rolled at a reduction of at least 85 percent.

10. An improvement according to claim 7, wherein the hot rolled band is cold rolled without an intermediate anneal between hot rolling and cold rolling.

11. An improvement according to claim 7, wherein the hot rolled band is annealed at a temperature of from 1400° - 1700°F prior to being cold rolled.

12. An improvement according to claim 11, wherein said annealed hot rolled band is cooled at a rate equivalent to a still air cool prior to being cold rolled.

\* \* \* \* \*

25

30

35

40

45

50

55

60

65